

## UNITED STATES PATENT OFFICE

2,575,219

## FERROUS ALLOYS AND ABRASIVE-RESISTANT ARTICLES MADE THEREFROM

David J. Giles, Latrobe, Pa., assignor to Latrobe Electric Steel Company, Latrobe, Pa., a corporation of Pennsylvania

No Drawing. Application January 10, 1951,  
Serial No. 205,441

15 Claims. (Cl. 75—126)

1

This invention relates to ferrous alloys and in particular to ferrous alloys having high resistance to abrasion. There has long been a need for steels having a materially greater resistance to abrasion than those commercially available and at the same time being easy to form, easy to grind and having good impact strength, i. e., ability to withstand shock. A good example is steel for use in the fabrication of router and shaper bits and lathe tools for the woodworking industry, and for other articles which are subject to considerable abrasion and shock and are thereby rapidly worn to a point where they can no longer meet required tolerances in the industry and must be resharpened, resurfaced or otherwise brought back to the tolerances of the industry.

In alloys for use in installations such as are described above in which the metal is subject to continual or recurring abrasion and impact, it is desirable that they be forgeable and hardenable and yet resist the action of abrasive substances and the shock of intermittent impacts. Historically, the search for alloys having certain desirable properties has lead to various combinations of alloying elements including combinations with vanadium. I have found, however, that while the general trend in vanadium alloys of steel has been in the direction of greater hardenability this is not alone the answer to the problem of abrasion resistance, and this is especially true when resistance to shock is also required.

I have discovered certain alloys having satisfactory forgeability and hardenability which can be made abrasive-resistant by properly controlling the carbon and vanadium content in a manner described in my copending application Serial No. 118,448, filed September 28, 1949, now abandoned, of which this is a continuation-in-part, without materially altering their forgeability and hardenability. One of these alloys is the subject of United States patent application Serial No. 91,002, filed May 2, 1949, now abandoned.

My present invention provides an abrasion-resistant alloy in which carbon, within certain limits, is added in excess of that necessary to give the alloy the desired forging and hardening characteristics and vanadium is added in an amount, again within certain limits, such that the ratio of the vanadium in excess of about 1% to the aforementioned excess of carbon is about 4.2:1.

Considering only the essential elements of my alloy, the preferred analysis for most combined abrasion and shock resisting applications is:

2

|                                                                          | Per cent |
|--------------------------------------------------------------------------|----------|
| C                                                                        | 1.8      |
| Cr                                                                       | 5        |
| V                                                                        | 4        |
| Si                                                                       | 0.3      |
| Mn                                                                       | 0.7      |
| Mo                                                                       | 1.1      |
| Balance substantially iron with residual impurities in ordinary amounts. |          |

10 The composition of my alloy may, however, extend over a wider range and still retain its desirable abrasive resistance. It may include alloying elements such as nickel, tungsten and cobalt in restricted amounts without detrimentally affecting the ability of the alloy to resist abrasion. The composition may fall within the limits of the following range of concentrations of alloying elements.

|                                                                          |    |                |
|--------------------------------------------------------------------------|----|----------------|
| 20                                                                       | C  | 1.4%—4.25%     |
|                                                                          | Si | 1% maximum     |
|                                                                          | Mn | 1.5% maximum   |
|                                                                          | Cr | 4%—8%          |
|                                                                          | V  | 3%—13%         |
| 25                                                                       | Mo | Less than 1.5% |
|                                                                          | W  | Less than 3%   |
|                                                                          | Co | Less than 5%   |
|                                                                          | Ni | Less than 3%   |
| Balance substantially iron with residual impurities in ordinary amounts. |    |                |

30 While the alloy of this invention may fall within the range of concentrations of alloying elements just enumerated and still retain its desirable characteristics of abrasion resistance and ability to withstand shocks, it is desirable to limit the composition to a narrower range of alloying elements for most economical and effective use of the alloy. The preferred narrow range of concentration of alloying elements to produce the most effective combination of abrasion resistance, ability to withstand shock, forgeability, hardenability and economy is as follows:

|                                                                          | Per cent    |
|--------------------------------------------------------------------------|-------------|
| 45                                                                       | C 1.65—1.95 |
|                                                                          | Cr 4—6      |
|                                                                          | V 3—5       |
|                                                                          | Si 0.1—0.7  |
|                                                                          | Mn 0.2—0.9  |
| 50                                                                       | Mo 0.8—1.3  |
| Balance substantially iron with residual impurities in ordinary amounts. |             |

55 While I have given specific silicon and manganese ranges in the composition of my alloy, these concentrations are the concentrations which

normally result from the raw materials which I have used and may accordingly vary within reasonable limits depending upon the raw materials used.

By the expression "less than" followed by a percentage figure in this application when referring to molybdenum, nickel, tungsten and cobalt, I mean that the particular element may be present in an amount not to exceed the percentage concentration given. The presence of these elements is optional up to the amount specified in the ranges of composition given above.

The alloy is forgeable and is air hardening as well as being abrasive-resistant when molybdenum is included in the composition. If it is desired to produce an alloy having similar abrasion resistance and forgeability but at a reduced cost and for use where air hardening is not necessary, the molybdenum may be omitted without materially affecting the other desirable properties.

In order to illustrate the abrasive resistance of my new alloy several heats were made within the range of composition specified above for my new alloy. The abrasion resistance of the alloy of my present invention and of an alloy steel having similar forgeability and hardenability characteristics previously used in applications for which my new alloy is intended were compared with the abrasion resistance of an 18-4-1 high-speed steel taken as a standard of 100% abrasion. The results of these abrasion tests on forged and hardened pieces one inch in diameter are tabulated below along with a tabulation of chemical composition:

Table I

|                    | Per cent abrasion <sup>1</sup> |  |  |  |  |  |  |  |
|--------------------|--------------------------------|--|--|--|--|--|--|--|
| Alloy A (standard) | 100                            |  |  |  |  |  |  |  |
| Alloy B            | 207                            |  |  |  |  |  |  |  |
| Alloy C            | 23                             |  |  |  |  |  |  |  |

<sup>1</sup> Per cent removed by abrasion.

Table II

| Alloy | C    | Cr   | W     | V    | Mo   | Si   | Mn   |                           |
|-------|------|------|-------|------|------|------|------|---------------------------|
| A     | .74  | 4.10 | 18.00 | 1.10 | .30  | .25  | .25  | Balance substantially Fe. |
| B     | 1.02 | 5.25 | ----- | .25  | 1.10 | 0.30 | 0.70 | Do.                       |
| C     | 1.80 | 5.21 | ----- | 3.95 | 1.12 | 0.38 | 0.70 | Do.                       |

Abrasions tests were also made on modifications of alloy C within the broad limits of composition heretofore stated. The results of these abrasion tests and the composition of the test pieces are given in Tables III and IV below.

Table III

|              | Per Cent Abrasion <sup>1</sup> |
|--------------|--------------------------------|
| Alloy Mod. A | 37                             |
| Alloy Mod. C | 31                             |
| Alloy Mod. D | 42                             |
| Alloy Mod. H | less than 2                    |
| Alloy Mod. I | 60                             |
| Alloy Mod. J | 0                              |

<sup>1</sup> Per cent removed by abrasion as compared with alloy A.

Table IV

| Alloy  | C    | Si  | Mn  | Cr   | V     | Mo    | Ni    | W     | Co    |                           |
|--------|------|-----|-----|------|-------|-------|-------|-------|-------|---------------------------|
| Mod. A | 1.83 | .42 | .66 | 5.45 | 4.08  | 1.22  | 2.71  | ----- | ----- | Balance substantially Fe. |
| Mod. C | 1.91 | .38 | .57 | 5.22 | 4.38  | 1.19  | ----- | 2.48  | ----- | Do.                       |
| Mod. D | 1.87 | .57 | .65 | 5.92 | 3.95  | 1.31  | ----- | ----- | 4.58  | Do.                       |
| Mod. H | 3.55 | .47 | .58 | 5.10 | 11.92 | ----- | ----- | ----- | ----- | Do.                       |
| Mod. I | 1.84 | .59 | .66 | 7.40 | 4.22  | ----- | ----- | ----- | ----- | Do.                       |
| Mod. J | 4.15 | .63 | .73 | 7.40 | 12.76 | 1.32  | ----- | ----- | 3.02  | Do.                       |

Careful comparison of the composition of the test pieces and their resistance to abrasion shows the superiority of the alloy of my invention over the alloys now used for applications requiring abrasion resistance as well as its superiority over standard 18-4-1 high-speed steel. The alloy previously used has lost about nine times as much material as the preferred alloy (alloy C) of my invention while the high-speed steel standard shows more than four times as much loss of material as does my preferred alloy.

The economic importance of these results becomes more apparent when it is realized that not only has the alloy of my present invention lost less than 25% as much material as the 18-4-1 high-speed steel but it does not incorporate the costly percentage of alloying elements which appear in the high-speed steel. Moreover, the alloy of this invention is easier to form, easier to grind, and is able to withstand shock better than the alloys having a higher chromium content as exemplified by the alloy described in my application Serial No. 91,002 mentioned above. This new alloy therefore serves a new field of usefulness in which resistance to shock or impact is necessary or desirable along with resistance to abrasion.

Peculiarly, the addition of excess carbon and vanadium in excess of 1% in the ratio of 4.2% vanadium to 1% carbon although increasing the abrasion resistance to a remarkable extent has little or no effect on the forgeability or hardenability of my alloy over those same physical properties of an alloy without such excess carbon and vanadium. For example, the Rockwell C hardness of alloy C and alloy B are substantially identical, as are their forging properties. Their abrasive resistances, however, are sharply distinguished as illustrated in Table I. If, however, a marked departure from this ratio of 4.2:1 is made,

then a marked change in forgeability and hardenability occurs, the direction and extent of which depends upon the nature and extent of the departure from this ratio.

My researches indicate that when carbon and vanadium appear in the above described excess and ratio they modify the characteristics of the alloy by very desirably augmenting its abrasive resistance without masking or nullifying the other physical characteristics of the basic alloy. I believe that the extraordinary abrasive resistance of my alloy depends upon the formation of vanadium carbides which remain out of solution and accordingly do not affect the hardenability or forgeability of my alloy. While this theory seems to be consistent with observable facts, I do not

bind myself thereto. The fact is that, whatever the mechanism may be, the addition of carbon and vanadium in the above described proportions does produce an unexpected and unusual abrasive resistance which is of great technical importance.

While I have described and disclosed the preferred embodiment of my invention, it is to be understood that the invention is not so limited but may be otherwise embodied and practiced within the scope of the following claims.

I claim:

1. An abrasion-resisting alloy comprising about 1.65% to 1.95% of carbon, about 4% to 6% of chromium, about 0.1% to 0.7% of silicon, about 0.2% to 0.9% of manganese, about 3% to 5% of vanadium, and the balance substantially iron with residual impurities in ordinary amounts, in which alloy the vanadium in excess of about 1% is combined with carbon in a ratio of about 4.2:1.

2. An abrasion-resisting alloy comprising about 1.65% to 1.95% of carbon, about 4% to 6% of chromium, about 0.1% to 0.7% of silicon, about 0.2% to 0.9% of manganese, about 0.8% to 1.3% of molybdenum, about 3% to 5% of vanadium, and the balance substantially iron with residual impurities in ordinary amounts, in which alloy the vanadium in excess of about 1% is combined with carbon in a ratio of about 4.2:1.

3. An abrasion-resisting alloy comprising about 1.8% of carbon, about 5% of chromium, about 0.3% of silicon, about 0.7% of manganese, about 4% of vanadium, and the balance substantially iron with residual impurities in ordinary amounts, in which alloy the vanadium in excess of about 1% is combined with carbon in a ratio of about 4.2:1.

4. An abrasion-resisting alloy comprising about 1.8% of carbon, 5% of chromium, about 0.3% of silicon, about 0.7% of manganese, about 1.1% of molybdenum, about 4% of vanadium, and the balance substantially iron with residual impurities in ordinary amounts, in which alloy the vanadium in excess of about 1% is combined with carbon in a ratio of about 4.2:1.

5. An abrasion-resisting alloy having carbon in excess of that necessary to give it the desired hardenability characteristics comprising about 1.65% to 1.95% of carbon, about 4% to 6% of chromium, about 0.1% to 0.7% of silicon, about 0.2% to 0.9% of manganese, about 3% to 5% of vanadium, and the balance substantially iron with residual impurities in ordinary amounts, and in which the concentrations of vanadium and carbon within the given limits are adjusted so that the ratio of vanadium in excess of about 1% to the excess carbon is about 4.2:1.

6. An abrasion-resisting alloy having carbon in excess of that necessary to give it the desired hardenability characteristics comprising about 1.65% to 1.95% of carbon, about 4% to 6% of chromium, about 0.1% to 0.7% of silicon, about 0.2% to 0.9% of manganese, about 0.8% to 1.3% of molybdenum, about 3% to 5% of vanadium, and the balance substantially iron with residual impurities in ordinary amounts, and in which the concentrations of vanadium and carbon within the given limits are adjusted so that the ratio of vanadium in excess of about 1% to the excess carbon is about 4.2:1.

7. An abrasion-resisting alloy having carbon in excess of that necessary to give it the desired hardenability characteristics comprising about 1.8% of carbon, about 0.3% of silicon, about 0.7% of manganese, about 5% of chromium, about 4% of vanadium, and the balance substantially

iron with residual impurities in ordinary amounts, in which the concentrations of vanadium and carbon within the given limits are adjusted so that the ratio of vanadium in excess of about 1% to the excess carbon is about 4.2:1.

8. An abrasion-resisting alloy having carbon in excess of that necessary to give it the desired hardenability characteristics comprising about 1.8% of carbon, about 0.3% of silicon, about 0.7% of manganese, about 1.1% of molybdenum, about 5% of chromium, about 4% of vanadium, and the balance substantially iron with residual impurities in ordinary amounts, in which the concentrations of vanadium and carbon within the given limits are adjusted so that the ratio of vanadium in excess of about 1% to the excess carbon is about 4.2:1.

9. An abrasion-resisting article formed from a forgeable abrasion-resisting steel comprising about 1.65% to 1.95% of carbon, about 4% to 6% of chromium, about 0.1% to 0.7% of silicon, about 0.2% to 0.9% of manganese, about 3% to 5% of vanadium, and the balance substantially iron with residual impurities in ordinary amounts, in which alloy the vanadium in excess of about 1% is combined with carbon in a ratio of about 4.2:1, said article being characterized by a factor of hardenability and forgeability comparable to a steel having less than 1% vanadium and a carbon content less than said article by a value equal to about

the per cent vanadium in said article—1%

4.2

10. An abrasion-resisting article formed from a forgeable abrasion-resisting steel comprising about 1.65% to 1.95% of carbon, about 4% to 6% of chromium, about 0.1% to 0.7% of silicon, about 0.2% to 0.9% of manganese, about 0.8% to 1.3% of molybdenum, about 3% to 5% of vanadium, and the balance substantially iron with residual impurities in ordinary amounts, in which alloy the vanadium in excess of about 1% is combined with carbon in a ratio of about 4.2:1, said article being characterized by a factor of hardenability and forgeability comparable to a steel having less than 1% vanadium and a carbon content less than said article by a value equal to about

the per cent vanadium in said article—1%

4.2

11. An abrasion-resisting article formed from a forgeable abrasion-resisting steel comprising about 1.8% of carbon, about 5% of chromium, about 0.3% of silicon, about 0.7% of manganese, about 1.1% of molybdenum, about 4% of vanadium, the balance substantially iron with residual impurities in ordinary amounts in which alloy the vanadium in excess of about 1% is combined with carbon in a ratio of about 4.2:1, said article being characterized by factors of hardenability and forgeability comparable to a steel having less than 1% vanadium and a carbon content less than said article by a value equal to about

the per cent vanadium in said article—1%

4.2

12. An article formed of forgeable abrasion-resisting steel having carbon in excess of that necessary to give it the desired hardenability characteristics comprising about 1.65% to 1.95% of carbon, about 4% to 6% of chromium, about 0.1% to 0.7% of silicon, about 0.2% to 0.9% of manganese, about 0.8% to 1.3% of molybdenum,

about 3% to 5% of vanadium, and the balance substantially iron with residual impurities in ordinary amounts and in which the concentrations of vanadium and carbon within the given limits are adjusted so that the ratio of vanadium in excess of about 1% to the excess carbon is about 4.2:1, said article being characterized by factors of hardenability and forgeability comparable to a steel having less than 1% vanadium and a carbon content less than said article by a value equal to about

the per cent vanadium in said article—1%

4.2

13. An abrasion-resisting alloy comprising about 1.4% to 4% of carbon, about 4% to 8% chromium, about 3% to 13% vanadium, about 1% maximum silicon, about 1.5% maximum manganese, less than about 1.5% molybdenum, less than about 3% nickel, less than about 3% tungsten, less than about 5% cobalt and the balance substantially iron with residual impurities in ordinary amounts, in which alloy the vanadium in excess of about 1% is combined with carbon in a ratio of about 4.2:1.

14. An abrasion-resisting alloy having carbon in excess of that necessary to give it the desired hardenability characteristics comprising about 1.4% to 4% of carbon, about 4% to 8% chromium, about 3% to 13% vanadium, about 1% maximum silicon, about 1.5% maximum manganese, less than about 1.5% molybdenum, less than about 3% tungsten, less than about 5% cobalt and the balance substantially iron with residual impurities in ordinary amounts, and in which the

10

20

25

30

35

concentrations of vanadium and carbon are adjusted so that the ratio of vanadium in excess of about 1% to the excess carbon is about 4.2:1.

15. An abrasion-resisting article formed of abrasion resisting steel having carbon in excess of that necessary to give it the desired hardenability characteristics comprising about 1.4% to 4% carbon, about 4% to 8% chromium, about 3% to 13% vanadium, about 1% maximum silicon, about 1.5% maximum manganese, less than about 1.5% molybdenum, less than about 3% tungsten, less than about 5% cobalt and the balance substantially iron with residual impurities in ordinary amounts, and in which the concentrations of vanadium and carbon within the given limits are adjusted so that the ratio of vanadium in excess of about 1% to the excess carbon is about 4.2:1, said article being characterized by high resistance to abrasion and by forging and hardening characteristics comparable to steels having a carbon content less than that of the article by an amount equal to the

the per cent vanadium—1%

4.2

DAVID J. GILES.

#### REFERENCES CITED

The following references are of record in the file of this patent:

#### FOREIGN PATENTS

| Number  | Country | Date          |
|---------|---------|---------------|
| 832,703 | France  | Oct. 3, 1938  |
| 834,198 | France  | Nov. 15, 1938 |